

# United States Patent [19]

Bourgois

[11] Patent Number: 4,818,631

[45] Date of Patent: Apr. 4, 1989

[54] STRAND FOR APPLICATION AS REINFORCEMENT IN OBJECTS OF POLYMER MATERIAL AS WELL AS ONE OR MORE SUCH STRAND COMPRISING OBJECTS OF POLYMER MATERIAL

[75] Inventor: Luc Bourgois, Desselgem, Belgium

[73] Assignee: N.V. Bekaert S.A., Zwevegem, Belgium

[21] Appl. No.: 48,619

[22] Filed: May 11, 1987

[30] Foreign Application Priority Data

Jun. 19, 1986 [NL] Netherlands ..... 8601599

[51] Int. Cl. 4 ..... B32B 15/00; B23P 17/06

[52] U.S. Cl. ..... 428/605; 57/902; 152/527; 428/377; 428/379; 428/683

[58] Field of Search ..... 428/364, 373, 379, 644, 428/615, 683, 605; 57/902, 216, 220

[56] References Cited

U.S. PATENT DOCUMENTS

3,977,174 8/1976 Boileau ..... 57/216 X  
4,176,705 12/1979 Russell et al. ..... 57/220 X  
4,258,543 3/1981 Canevari et al. ..... 57/902 X  
4,268,573 5/1981 Baillievier ..... 57/902 X  
4,328,852 5/1982 Poque et al. ..... 57/902 X

## FOREIGN PATENT DOCUMENTS

0144811 of 0000 European Pat. Off. .

## OTHER PUBLICATIONS

Research Disclosure, No. 184, Augustus 1979, blz. 430-431, No. 18441, Industrial Opportunities Ltd., Homewell Havant, Hampshire, GB; "Rubber Articles Reinforced with High Tensile Steel Cord".

Primary Examiner—Lorraine T. Kendall  
Attorney, Agent, or Firm—Foley & Lardner, Schwartz, Jeffery, Schwaab, Mack, Blumenthal & Evans

[57] ABSTRACT

A strand for reinforcing objects made of polymer material comprising at least one core wire and less than six outside wires arranged round it, the core wire having an outside diameter larger than the diameter of the circle tangent to each of the outside wires in the hollow space that remains free when their cross-sections have the highest packing density and smaller than the diameter of the outside wires, whereby the outside wires are made of carbon steel wire with a tensile strength of at least  $2250-1130 \log d \text{ N/mm}^2$ , d being the wire diameter in mm. The core wire has a tensile strength less than  $2250-1130 \log d \text{ N/mm}^2$ .

5 Claims, 1 Drawing Sheet



ab~~FIG: 2.~~ab~~FIG: 2.~~

**STRAND FOR APPLICATION AS  
REINFORCEMENT IN OBJECTS OF POLYMER  
MATERIAL AS WELL AS ONE OR MORE SUCH  
STRAND COMPRISING OBJECTS OF POLYMER  
MATERIAL**

The invention relates to a strand for application as reinforcement in objects of polymer material comprising a core wire and outside wires arranged round it, the core having an outside diameter that is larger than the diameter of the circle tangent to each of the outside wires in the hollow space that remains free when their cross-sections have the highest packing density and that is smaller than the diameter of the outside wires.

Such strand is known from Belgian Pat. No. 834,259 of the present applicant wherein a strand for the reinforcement or strengthening of polymer material is described. Such strand consists of a core and outside wires arranged round it, the core being given such an outside diameter that between the outside wires gaps are created whereinto polymer material can penetrate during the embedding process, thereby greatly enhancing the bond between the strand material and the polymer material. The core can consist of one core wire or of one core strand, which is then formed from several core wires.

The term of "highest packing density" stated hereinbefore is in this case to be understood as referring to a two-dimensional configuration of cross-sections of the outside wires, such that each separate outside wire is in contact with two adjacent outside wires, the centres of all adjacent cross-sections lying on the circumference of a circle. The inside tangent-circle diameter of the hollow space thus enclosed by the stacked cross-sections which serves as minimum diameter for the outside diameter of the core to be used can be determined easily.

Such strands are widely applied in all kinds of objects of polymer material such as synthetic conveyor belts and rubber vehicle tyres.

The strands according to Belgian Pat. No. 834,259 applied heretofore have the disadvantage that, with minimal diameters of core wire and outside wires as regards strand strength, the polymer penetration is often still insufficient. To enhance this penetration, either the diameter of the outside wires should be reduced or the diameter of the core wire enlarged. Both solutions are, however, unattractive from which follows that the strength of the strand and the extent of polymer penetration are conflicting properties.

The present invention is intended to provide a solution to the disadvantage discussed hereinabove and relates for that purpose to a strand as described hereinbefore characterised in that the outside wires are made of carbon steel wire with a tensile strength of at least 2250-1130 d N/mm<sup>2</sup>, d being the wire diameter in mm.

The outside wires are preferably made of carbon steel wire with a tensile strength of at least 2325-1130 log d N/mm<sup>2</sup>, d being the wire diameter in mm.

For an explanation of the tensile-strength formula stated hereinbefore, the reader is referred to European Patent Application No. 0 144 811 of the present applicant, wherein a description is given of carbon steel wire with high tensile strength meeting such requirements.

The application of aforementioned carbon steel wire with high tensile strength has the advantage that outside wires of a smaller diameter than usual heretofore will suffice for an equal tensile strength of the total strand,

which results in a considerable increase in rubber penetration, the total tensile strength being equal. Further, as a result of the possibility to use outside wires of a smaller diameter, the total diameter of the strands is reduced, which, compared to the strands used heretofore, has the advantage of an enhanced rubber penetration on the one hand and on the other hand the advantage of a reduced total strand diameter which shows itself in a decrease in the thickness of the polymeric objects whereinto such strands are incorporated.

The high tensile wire used for the strands described hereinbefore can be obtained in various ways.

This wire can for instance be obtained departing from carbon steel wire with high carbon content subject to

15 the observation of special precautions, such as a choice or wire rods with few impurities (inclusions, residual and/or scrap elements) and refined manufacturing methods, for instance wire drawing with small sub-reductions (increase in the number of drawing passes).

20 However, this does not always offer high tensile wire that can be successfully processed into strands during bunching or cabling. This wire can also be obtained departing from high carbon steel wire with the usual silicon and manganese contents, if only a sulfur content of not more than 0.015 per cent by weight is allowed, and preferably a sulphur content that is lower than 0.010 per cent by weight, as described in aforementioned European Patent Application No. 0 144 811.

Preferably, the core of the strand according to the invention is one core wire. The core can also consist of one core strand, which is then composed of several core wires, for instance obtained by bunching or cabling in the usual way.

With particular advantage, the core wire or the core wires constituting the core receive a regular undulatory deformation in longitudinal direction. Such undulatory deformation is described in Belgian Pat. No. 861.243 of the present applicant and has the advantage that such core is far less sensitive to rupture than a core used in the normal way that is not provided with deformations.

40 In a very advantageous embodiment of the strand according to the invention, the core wire is or the core wires constituting the core are made of a carbon steel with a tensile strength smaller than 2250-1130 log d N/mm<sup>2</sup>, d being the wire diameter in mm, such core with a lower tensile strength than indicated hereinabove with respect to the outside wires has a reduced rupture risk. The breaking elongation of such core wires with lower tensile strength is greater than the breaking elongation of a wire with higher tensile strength. If the core wires applied have a tensile strength smaller than 2250-1130 log d N/mm<sup>2</sup> and have, moreover, received an undulatory deformation in longitudinal direction, as indicated hereinbefore, a strand is obtained the core of which will remain intact even under very extreme load an bending, having a very favourable effect upon the operational life of the strand.

45 The core wire or the core wires constituting the core can also be suitably made of carbon steel with a tensile strength of at least 2250-1130 log d N/mm<sup>2</sup>, preferably at least 2325-1130 log d N/mm<sup>2</sup>, d being the wire diameter. Such type of strand is important when extremely high tensile loads are applied to the strand, while the bending loads are kept lower.

50 For certain applications, the strand core does not have to be made of carbon steel wire. For applications in which the core is subjected to strongly varying bending loads it may be advantageous that the core wire or

the core wires constituting the core consist of a synthetic monofilament.

In that case, the type of synthetic material chosen will suitably have a good deformation resistance, so that the polymer penetration between the outside wires is always maintained. Synthetic materials applicable for the monofilaments are for instance : polyamide, polyester and, in particular, para-phenylene terephthalic amide.

The invention also relates to objects of polymer material, these objects being reinforced with one or more strands according to the invention.

The invention particularly relates to a rubber vehicle tire comprising a carcass and at least one belt, reinforced with strands of carbon steel wire. Such rubber tire is characterised according to the invention in that the carcass and/or the belt are reinforced with strands according to the invention. Such strand to be used for the carcass and/or the belt can for instance be composed of one core wire and four outside wires arranged round it. Assuming that the outside wires have a diameter of for instance 0.25 mm, calculations show that, if the four outside wires are applied with the highest packing density, a wire with a diameter of 0.10 mm will fit the hollow space which remains free inside the outside wires. A core wire with a diameter of 0.15 mm will then be chosen, for instance, to obtain the required rubber penetration. If all wires were made of carbon steel that has not been drawn to high tensile strength (in other words, wires with a tensile strength of not more than 2250-1130  $\log d$  N/mm<sup>2</sup>,  $d$  being the wire diameter in mm), the strength required for the strand would be attained with a strand composed of a core wire of 0.15 mm and four outside wires of 0.25 mm arranged round it. If the outside wires are made of carbon steel that is drawn to high tensile strength (in other words, with a tensile strength of at least 2250-1130  $\log d$  N/mm<sup>2</sup>, preferably 2325-1130  $\log d$  N/mm<sup>2</sup>), the diameter of the outside wires can be reduced from 0.25 to 0.23 mm for a strand with equal strength. By this reduction in the diameter of the outside wires, the core wire diameter being equal, a considerable increase in rubber penetration is attained with the same strand strength. If desired for certain purposes, the core wire can also be constituted by a core wire of carbon steel that is drawn to high tensile strength, or, alternatively, by a core wire consisting of a synthetic monofilament.

In order to attain optimal properties, the core wire has further received a regular undulatory deformation in longitudinal direction as described hereinbefore.

Dependent on the purpose of the strands, a choice will be made with respect to the wire diameters to be used.

For passenger car tires, for instance, a core wire of 0.12 mm and 0.20 mm dia outside wires arranged round it will be most satisfactory for the formation of the tyre carcass.

For the belt or belts present in the tires, a wire of 0.138 or 0.15 mm can be applied advantageously as core wire and wires of 0.23 or 0.25 mm as outside wires. The material of the core wire and of the outside wires can be chosen within the scope of the invention as indicated hereinbefore.

For application in truck tires, when strands are used for the carcass, it will be possible to use the same strands indicated hereinbefore for the passenger car tires, too. An excellent result will be obtained for the belt if a diameter is chosen of from 0.18 up to 0.21 mm for the core wires and of from 0.30 up to 0.35 mm for the out-

side wires ; the types of material again being chosen from the types according to the invention described hereinbefore.

The numerical values indicated hereinbefore are solely meant as example and do not restrict the invention in any way.

The invention will hereinafter be illustrated with the help of the accompanying drawing, wherein :

FIGS. 1a and 1b represent a couple of outside wire arrangements with the highest packing density and

FIGS. 2a and 2b represent the outside wires from FIGS. 1a and 1b after the application of a core wire.

FIG. 1a represents four outside wires 1 with the highest packing density. A dotted line indicates the tangent circle in the hollow space left free by the four wires 1, which each time corresponds to the minimum value of the core wire 2 to be applied for these outside wires. In FIG. 1b such highest packing density of outside wires is indicated for application of three outside wires 1. Here again, a dotted line indicates the circle diameter of which corresponds to the minimum value of the diameter of the core wire 2 to be applied for this arrangement.

FIG. 2a represents the outside wires of FIG. 1a in a configuration wherein the core wire 2 is surrounded by the outside wires 1. Giving the core wire 2 a diameter larger than the minimum diameter represented in FIG. 1a provides an enhanced penetration capacity for the polymer material between the outside wires 1.

FIG. 2b represents the same situation for a strand consisting of one core wire 2 and three outside wires 1 as in the original form sketched in FIG. 1b.

Here follow some specific values of a strand according to the invention ( $1 \times 0.15 + 4 \times 0.23$ ) and of a state-of-the-art ( $1 \times 0.15 + 4 \times 0.25$ ) ; the total tensile strength of both strands being nearly equal :

| Strand                   | Tensile strength (Newton) | Diameter (mm) | Openness (%) |
|--------------------------|---------------------------|---------------|--------------|
| acc. to invention        | 571 N                     | 0.61 mm       | 17.23        |
| acc. to state of the art | 570 N                     | 0.65 mm       | 14.04        |

To determine the openness (%) of a strand, a circle is drawn centred on the centre of the core and passing through the centres of the outside wires (see FIG. 2a). The openness is the proportion of the sum of the lengths (AB; CD; EF; GH) between the outside wires to the total circumference of the circle.

I claim:

1. A strand for reinforcing objects made of polymer material comprising a core comprising at least one wire and at least three but less than six outside wires arranged round it, the core wire having an outside diameter larger than the diameter of the circle tangent to each of the outside wires in the hollow space that remains free when their cross-section have the highest packing density and smaller than the diameter of the outside wires, wherein the outside wires are made of carbon steel wire with a tensile strength of at least 2250-1130  $\log d$  N/mm<sup>2</sup>,  $d$  being the wire diameter in mm, said core wire being made of carbon steel with a tensile strength less than 2250-1130 d N/mm<sup>2</sup>.

2. The strand according to claim 1 wherein the outside wires are made of carbon steel wire with a tensile

strength of at least 2325-1130 d N/mm<sup>2</sup>, d being the wire diameter in mm.

3. The strand according to claim 1 wherein the core is a single wire.

4. The strand according to claim 1 wherein the core is a strand composed of several wires.

5. The strand according to claim 1 wherein the core has an undulatory deformation in the longitudinal direction.

\* \* \* \* \*

10

15

20

25

30

35

40

45

50

55

60

65

UNITED STATES PATENT AND TRADEMARK OFFICE  
CERTIFICATE OF CORRECTION

PATENT NO. : 4,818,631

DATED : April 4, 1989

INVENTOR(S) : Luc BOURGOIS

It is certified that error appears in the above-identified patent and that said Letters Patent is hereby corrected as shown below:

Column 1, line 10, "rount" should be --round--;  
Column 2, line 16, "or" should be --of--;  
line 44, "small" should be --smaller--;  
line 45, "such" should be --Such--.

Signed and Sealed this  
Twenty-first Day of November, 1989

*Attest:*

JEFFREY M. SAMUELS

*Attesting Officer*

*Acting Commissioner of Patents and Trademarks*